

Aug. 1, 1967

L. V. ABRAMS ET AL

3,333,365

THROWING WHEEL VANE AND METHOD OF MANUFACTURE THEREOF

Filed Oct. 22, 1964

2 Sheets-Sheet 1

*Fig. 1.*



*Fig. 2.*



INVENTORS

*Louis V. Abrams*  
*Ralph W. Moore*

BY *Connolly and Gutz*  
ATTORNEYS

Aug. 1, 1967

L. V. ABRAMS ET AL

3,333,365

THROWING WHEEL VANE AND METHOD OF MANUFACTURE THEREOF

Filed Oct. 22, 1964

2 Sheets-Sheet 2



INVENTORS  
Louis V. Abrams  
Ralph W. Moore  
BY Connolly and Hutz  
ATTORNEYS

1

3,333,365

## THROWING WHEEL VANE AND METHOD OF MANUFACTURE THEREOF

Louis V. Abrams and Ralph W. Moore, Hagerstown, Md., assignors to The Pangborn Corporation, Hagerstown, Md., a corporation of Delaware

Filed Oct. 22, 1964, Ser. No. 405,730  
9 Claims. (Cl. 51—9)

The present invention relates to both a method for making a vane and a vane for use in a throwing wheel for projecting streams of particles against work pieces to subject the work pieces to cleaning, abrading or peening action or the like. A typical wheel of this kind is shown in U.S. Patent 2,869,289, granted Jan. 20, 1959, and in U.S. Patent 3,151,417 granted Oct. 6, 1964.

Among the objects of the present invention is the provision of improved vanes for the above wheels, as well as improved methods for making such vanes.

Other objects and advantages of the present invention will become more apparent from a study of the following description and drawings wherein:

FIG. 1 is a horizontal section of a mold for casting the vanes according to the present invention;

FIG. 2 is a vertical section of the mold of FIG. 1 taken along line 2—2; and

FIG. 3 is a schematic view of the steps involved in producing a vane in accordance with this invention.

When used in the above type of throwing wheels, the vanes gradually wear away in view of the eroding action of the abrasive particles, the particles are very hard, such as steel. The movement of the particles along and against the length of the vane causes erosion of the vane surfaces. In some very heavy usages as when sand or alumina contaminate the particles, the vanes might have to be replaced after only about twenty hours of operation or less.

It has been discovered that this wear or erosion starts at any surface imperfection. For example, even the minute indentations resulting from the Rockwell hardness tests are starts of accelerated wear, although a magnifying glass is necessary to see these minute indentations or impressions. Accordingly by the present invention, throwing wheel vanes of improved wear resistance are cast and surface ground below the depth of the deepest roughness to provide a vane which is smooth and flat. To further resist wear the vanes may also be tempered in addition to being surface ground.

Applicant's invention is a distinct departure from prior practices in that heretofore vanes were surface ground primarily for esthetic reason, to give the vanes a more pleasant appearance and to dress the shape to the final specification. However, there was never any recognition that if the vanes were actually ground as flat and smooth as possible, increased wear life would result. Consequently, no conscious effort was made to finish the vanes to such an extent that they were ground below the depth of the deepest roughness resulting from the casting process, so as to increase the wear life. In fact, it was generally believed that ground surfaces would erode much more

2

rapidly and would cause premature breakage by, for example, developing fine cracks.

FIGS. 1 and 2 illustrate one effective casting technique that produces a plurality of vanes 86, 87 from each mold. The above vanes 86, 87 are readily made, for example, with an ordinary sand casting mold with the gating provided by a baked sand insert shaped to provide the desired base bottom configuration. The gating is preferably arranged to have a constriction adjacent the recessed lower surface 82 of the vane so that when the casting is completed and the solidified metal is withdrawn from the mold, the gate can be readily broken off and will then break close to that surface. Although the vane can tolerate a small amount of gate material projecting out from surface 81, a  $\frac{1}{2}$  square inch cross-section gate will generally break off quite close where the dovetail 85 is fairly massive. Particularly good breaking takes place where the gate is made relatively thin, for example  $\frac{1}{2}$  inch in width, the desired area being provided by having the gate extend the necessary length along surface 81. The vanes can either be cast one at a time, or a plurality can be cast together by running their respective gates to a common pour opening or riser.

FIGS. 1 and 2 show one technique for producing a plurality of these vanes. A mold is here shown as two vanes 86 and 87 using sand filling 88 with a baked core insert 90 providing gates 91, runners 92, and expansion domes 93. The pouring takes place through riser 94. After casting is completed vanes 86 and 87 are removed from the mold and the risers and gates 91 are broken off.

Vanes 86 and 87 are preferably of abrasion-resistant heat treated alloy carbon containing the following composition by percentage of weight:

|    | Percent |
|----|---------|
| C  | 3.3     |
| Si | 0.46    |
| Cr | 16.3    |
| Mo | 2.92    |
| Fe | Balance |

After being cast the vanes are then heat treated or subjected to a hardening technique by being treated for about one hour at a temperature of approximately 1750° F. followed by air quenching.

Advantageously, the surface hardness of vanes 86 and 87 is in the range of from Rc 63 to 68. This hardness range is particularly desirable because harder faces do not add to the wear life and are susceptible to cracking and chipping, while a face hardness below Rc 63 reduces the wear life.

The following tables illustrate the wearability of dry sand cast vanes which were treated to 1750° F. and air quenched. All of the vanes have the following composition by percentage weight:

|         |    |
|---------|----|
| 3.3%    | C  |
| 0.46%   | Si |
| 16.3%   | Cr |
| 2.92%   | Mo |
| Balance | Fe |

TABLE I

| Vane Type             | Orig. Wt. in Grams | Wt. at End of 3 Hrs. | Gram Loss | Wt. at End of 4 Hrs. | Gram Loss | Wt. at End of 15 Hrs. | Gram Loss | Gram Loss Per Hour |
|-----------------------|--------------------|----------------------|-----------|----------------------|-----------|-----------------------|-----------|--------------------|
| Normal-1              | 1,459              | 1,455                | 4         | 1,453                | 6         | 1,434                 | 25        | 1.67               |
| Normal-2              | 1,456              | 1,451                | 5         | 1,450                | 6         | 1,424                 | 32        | 2.13               |
| Tempered and Ground-1 | 1,365              | 1,362                | 3         | 1,360                | 5         | 1,336                 | 29        | 1.90               |
| Tempered and Ground-2 | 1,364              | 1,360                | 4         | 1,358                | 6         | 1,328                 | 36        | 2.40               |
| Ground-1              | 1,382              | 1,379                | 3         | 1,377                | 5         | 1,357                 | 25        | 1.67               |
| Ground-2              | 1,383              | 1,380                | 3         | 1,379                | 4         | 1,363                 | 20        | 1.33               |

TABLE II.—SUMMARY OF RESULTS

| Vane Type           | Gram Loss Per Hour |                  |                   |
|---------------------|--------------------|------------------|-------------------|
|                     | At End of 3 Hrs.   | At End of 4 Hrs. | At End of 15 Hrs. |
| Normal              | 1.5                | 1.5              | 1.90              |
| Tempered and Ground | 1.17               | 1.38             | 2.17              |
| Ground              | 1.0                | 1.13             | 1.50              |

TABLE III

| Vane Type | Orig. Wt. | Wt. At 10½ Hrs. | Gram Loss | Wt. At 100 Hrs. | Gram Loss | Gram Loss Per Hr. |
|-----------|-----------|-----------------|-----------|-----------------|-----------|-------------------|
| Normal-1  | 1,436     | 1,413           | 23        | 1,271           | 165       | 1.65              |
| Normal-2  | 1,437     | 1,412           | 25        | 1,240           | 197       | 1.97              |
| Ground-1  | 1,408     | 1,388           | 20        | 1,241           | 167       | 1.67              |
| Ground-2  | 1,407     | 1,389           | 18        | 1,243           | 164       | 1.64              |

TABLE IV

| Vane Type | Gram Loss Per Hour |                    |
|-----------|--------------------|--------------------|
|           | At End of 10 Hrs.  | At End of 100 Hrs. |
| Normal    | 2.29               | 1.81               |
| Ground    | 1.81               | 1.66               |

As is evident from Tables I and II, although the rate of wear of conventional sand cast vanes is eventually the same as sand cast vanes which are tempered and ground, tempering the vane after grinding does effectively delay the start of wear. In fact, although not apparent from Tables I and II, at the end of the first hour of testing, the tempered ground face vanes even showed somewhat less wear than the untempered ground face vanes. Tables I-IV also clearly indicate that the sand cast vanes which are ground smooth and flat have an appreciably greater wear life than normal or conventional vanes.

Although ground sand cast vanes are particularly desirable in extending vane life, vanes which are chill cast and surface ground have about a three-to-one longer wear life than the sand cast vanes. The following tables illustrate a comparison of sand cast and chill cast vanes.

TABLE V

| Vane Type              | Orig. Wt. in Grams | Wt. at 10½ Hrs. | Gram Loss | Wt. at 100 Hrs. | Gram Loss |
|------------------------|--------------------|-----------------|-----------|-----------------|-----------|
| Normal Sand Cast No. 1 | 1,436              | 1,413           | 23        | 1,271           | 165       |
| Normal Sand Cast No. 2 | 1,437              | 1,412           | 25        | 1,240           | 197       |
| Ground Sand Cast No. 1 | 1,408              | 1,388           | 20        | 1,241           | 167       |
| Ground Sand Cast No. 2 | 1,407              | 1,389           | 18        | 1,243           | 164       |
| Chill Cast No. 1       | 1,422              | 1,414           | 8         | 1,389           | 63        |
| Chill Cast No. 2       | 1,405              | 1,397           | 8         | 1,343           | 62        |

TABLE IV.—SUMMARY OF RESULTS

| Vane Type        | Gram Loss Per Hour |                    |
|------------------|--------------------|--------------------|
|                  | At End of 10½ Hrs. | At End of 100 Hrs. |
| Normal Sand Cast | 2.29               | 1.81               |
| Ground Sand Cast | 1.81               | 1.66               |
| Chill Cast       | 0.76               | 0.625              |

The improved results of chill cast vanes over sand cast vanes might be understood from the difference in their microstructures. For example, sand cast and heat treated vanes have a predominance of larger grain (Cr, Mo)  $Fe_3C$  surrounded by tempered martensitic matrix. The carbides

are singular islands, each surrounded by the tough, high strength martensite which has secondary carbides imparting further hardness within the individual grains and grain boundaries. The micro-structure of chill cast and heat

5 treated vanes, however, has a predominance of fine, extremely hard, brittle (Cr, Mo)  $Fe_3C$  with a martensitic matrix. The carbides are acicular or needle-like and are coupled in an inter-connected cleavage pattern (dendritic) which indicates a high overall hardness with high brittleness and low overall strength.

10 Despite the fact that chill cast vanes give such outstanding results, sand cast vanes are more desirable for large scale use. The main disadvantage with chill cast vanes is the lack of uniformity in production lots. Casting 15 defects predominate the production of the chill cast vanes. Although the best vanes from a large quantity of chill 20 cast vanes would have a wear life three times longer than that of sand cast vanes, the uniformity of production of sand cast vanes makes these vanes more desirable.

25 FIG. 3 schematically illustrates the method of this invention. As indicated therein after the sand casting step 106 or the chill casting step 108, the vane is ground at grinding station 110, is then heated at heat station 112, and then quenched at quenching station 114. The resultant 30 vane 100 includes its cast body 102 having a smooth ground abrasive propelling face 104. As indicated above the hardness may advantageously be in the range of from Rc 63 to 68 Rockwell.

35 Obviously, many modifications and variations of the present invention are possible in light of the above teachings. It is, therefore, to be understood that within the scope of the appended claims the invention may be practiced otherwise than as specifically described.

What is claimed is:

35 1. The method of making an abrasive throwing vane having an abrasive propelling face for an abrasive throwing wheel which method consists essentially of the steps of casting a vane, and grinding the surface of said face below the depth of the deepest roughness of said face resulting from said casting step to make said surface smooth and flat.

2. The method of claim 1 including the step of hardening said vane after it has been ground.

3. The method of claim 1 wherein said step of casting comprises sand casting said vane.

4. The method of claim 3 including the step of hardening said vane after it has been ground.

5. The method of claim 4 wherein said step of hardening includes heating said vane to approximately 1750° F. and air quenching said vane.

6. The method of claim 1 wherein said step of casting comprises chill casting said vane.

7. The method of claim 6 including the step of hardening said vane after it has been ground.

55 8. The method of claim 7 wherein said step of hardening includes heating said vane to approximately 1,750° F. and air quenching said vane.

9. A throwing vane having a cast body, an abrasive propelling face on said body, said face having a smooth ground surface, said vane being hardened and having a Rockwell hardness number in the range of from Rc 63 to 68.

60 10. The method of claim 1 wherein said step of casting comprises chill casting said vane.

11. The method of claim 7 wherein said step of hardening includes heating said vane to approximately 1,750° F. and air quenching said vane.

12. The method of claim 9 including the step of hardening said vane after it has been ground.

13. The method of claim 10 including the step of hardening said vane after it has been ground.

14. The method of claim 12 including the step of hardening said vane after it has been ground.

15. The method of claim 13 including the step of hardening said vane after it has been ground.

#### References Cited

##### UNITED STATES PATENTS

|           |         |                |          |
|-----------|---------|----------------|----------|
| 1,736,495 | 11/1929 | Graff          | 29—529   |
| 2,077,636 | 4/1937  | Minich         | 51—9     |
| 2,134,749 | 11/1938 | Burt           | 29—529 X |
| 2,204,633 | 6/1940  | Turnbull       | 51—9     |
| 2,314,069 | 3/1943  | Blount         | 51—9     |
| 2,376,639 | 5/1945  | Unger          | 51—9     |
| 2,869,289 | 1/1959  | Gossard        | 51—9     |
| 3,151,417 | 10/1964 | Hartman et al. | 51—9     |